

1

2,944,024

## LUBRICANTS CONTAINING FATTY ACID ESTERS OF SACCHARIDES

Arnold J. Morway, Clark, and Walter E. Waddey, Westfield, N.J., assignors to Esso Research and Engineering Company, a corporation of Delaware

No Drawing. Filed Mar. 28, 1958, Ser. No. 724,524

7 Claims. (Cl. 252—40.5)

This invention relates to lubricating compositions. Particularly, it relates to lubricating oil compositions which are thickened with an ester of a saccharide and a high molecular weight monocarboxylic acid.

It has been found that esters of disaccharides and high molecular weight fatty acids can be dispersed in lubricating oils to form semi-fluid greases having excellent stability against separation. Furthermore, the use of these esters as thickeners makes possible the preparation of non-metallic lubricants and because of their non-poisonous effect they may be used in those applications where a non-poisonous lubricant is required. For example, such ester thickeners may be used to prepare lubricants for use in food handling equipment such as dough mixers, conveyors, bottling, packaging and canning equipment. They may also be used in those applications where an ash-less lubricant is desired. It has been further found that lubricants containing the ester as a thickening agent are compatible with soap, salt and soap-salt materials, and can thus be further modified by the incorporation of these other materials. For example, by the addition of a minor quantity of calcium acetate, the dropping point of the ester base grease may be materially increased and its anti-wear properties are improved. Still, other properties may be built into the ester lubricant, depending upon the choice of additive material incorporated.

The disaccharide portion of the ester is selected from the group consisting of sucrose, maltose, lactose and cellobiose. The monocarboxylic acid portion of the ester can be derived from fatty acids containing 12 to 32, e.g. 16 to 24 carbon atoms. This includes naturally-occurring or synthetic, substituted and unsubstituted, saturated and unsaturated fatty acids. Examples of such acids include palmitic, stearic, dihydroxy stearic, behenic, montanic, linolinic, linoleic, arachidic, ricinoleic, oleic, hydrogenated fish oil, tallow acids, etc.

The esters which can be used as thickeners will include the mono-, di- and tri-esters. Specific examples of these esters include: sucrose mono-stearate, sucrose distearate, sucrose tristearate, maltose dipalmitate, maltose monolaurate, maltose dimelissate, cellobiose monooleate, sucrose monotallowate, etc. Particularly preferred because of their commercial availability in large quantities are the sucrose mono and distearate.

Semi-fluid greases may be prepared by dispersing 3 to 40, e.g. 5 to 30 wt. percent of the ester in a lubricating oil by heating the ester and oil mixture until the ester dissolves in the oil under stirring. This will generally occur at about 280° to 320° F. The composition is then allowed to cool without stirring, whereupon a smooth, homogeneous stable semi-fluid grease results. This composition may be used per se as a lubricant. If it is desired to make a more solid and higher dropping point grease, then other thickeners may be incorporated into the lubricant, or conversely, the ester may be used to modify other more conventional lubricants. Thus, the ester may be also incorporated into greases contain-

2

ing more conventional grease forming materials such as: soaps, soap-salt or mixed-salt complexes, polymeric thickeners (e.g. polymers of C<sub>2</sub> to C<sub>4</sub> monoolefins of 10,000 to 200,000 mol. wt. such as polyethylene), or inorganic thickeners (e.g. clay, carbon black, silica gel, etc.). The addition of the ester to such greases in minor amounts, e.g. 0.5 to 10.0 wt. percent, acts to prevent syneresis and accompanying oil separation. In these instances, the ester may be directly added to other greases and dispersed by slight heating; or a lubricating oil dispersion of the ester may be added to other greases; or the other thickeners may be added or formed in the lubricating oil dispersion of the ester.

A particularly desirable material for use with the ester thickeners are the alkaline earth metal (e.g. calcium, barium, strontium) salts of C<sub>2</sub> to C<sub>6</sub> fatty acids (acetic, propionic, butyric, etc.). Calcium acetate is particularly preferred for this purpose, since it will not only make a high dropping point solid grease, but will also impart considerable anti-wear and extreme pressure properties to the ester-containing lubricant. While the metal salts mentioned above may be added to the ester thickened lubricant in the form of an aqueous solution followed by dehydration, it is generally more desirable to form the alkaline earth metal salt in situ in the ester and oil mixture. This is readily accomplished by the reaction of an alkaline earth metal base, e.g. lime, with the desired acid, e.g. acetic acid or its anhydride. The mixture may or may not be externally heated depending upon what salt is formed and whether or not it is desired in the form of a hydrate. For example, if the salt formed is calcium acetate and if a small amount of water is present and the temperature of reaction is maintained below about 180–200° F. the dihydrate will form. Now if the same reaction mixture is heated above about 180–200° F. the monohydrate will form, while temperatures of about 300° F. will result in anhydrous calcium acetate. Either the hydrates or anhydrous form may be desirable depending upon the ultimate use. Thus, generally speaking, for low temperature operation the hydrates will result in the greatest thickening effect while the anhydrous form will have less thickening effect but will be more desirable for high temperature use. Usually about 5 to 40 wt. percent, e.g. 10 to 35 wt. percent of the alkaline earth metal salt may be advantageously used in the ester thickened oil.

The lubricating oil used in the compositions of the invention may be a mineral lubricating oil, a synthetic lubricating oil, or mixtures thereof. Synthetic lubricating oils which may be used include esters of dibasic acids (e.g. di-2-ethyl hexyl sebacate); esters of glycols (e.g. C<sub>18</sub> Oxo acid diester of tetraethylene glycol); complex esters (e.g. the complex ester formed by reacting one mole of sebacic acid with two moles of tetraethylene glycol and two moles of 2-ethyl-hexanoic acid); formals, silicones, carbonates, polyglycols and other synthetic lubricating oils known in the art.

Various other additives may also be added to the lubricating composition in amounts of about 0.1 to 10.0 weight percent, based on the total weight of the composition. Examples of such additives include: detergents such as calcium petroleum sulfonate; corrosion inhibitors such as sorbitan monooleate; pour depressants; dyes; still other grease thickeners and the like.

The invention will be further understood by the following examples which include preferred embodiments of the invention.

## Example I

18.0 wt. percent of sucrose mono-stearate was added to 82.0 wt. percent of a mineral oil having a viscosity of 55 SUS at 210° F. This mixture was then heated

while stirring to 300° F. in order to disperse the sucrose ester in the oil. The mixture was then allowed to cool quietly without stirring, and a stable semi-fluid grease composition resulted. The resulting composition was uniform, homogeneous, having an opaque appearance and an unworked ASTM penetration at 77° F. of 400 mm./10.

#### Example II

Example I was repeated, but using sucrose distearate in place of sucrose monostearate.

10

initiated until the temperature reached 220° F., at which point a sample was taken. The remainder of the composition was heated to 320° F. to completely dehydrate the calcium acetate, followed by cooling to 200° F. where phenyl- $\alpha$ -naphthylamine was added, then cooled to room temperatures.

The compositions prepared above and their physical characteristics are summarized in the following table:

TABLE  
Composition and properties of examples

|                                                                                    | I                                                   | II                                | III                              |                         | IV                      | A       |         |
|------------------------------------------------------------------------------------|-----------------------------------------------------|-----------------------------------|----------------------------------|-------------------------|-------------------------|---------|---------|
|                                                                                    |                                                     |                                   | 220° F.                          | 320° F.                 |                         | 320° F. | 220° F. |
| Composition (wt. percent):                                                         |                                                     |                                   |                                  |                         | 5.0%                    |         |         |
| Sucrose monostearate                                                               | 18.0%                                               | 18.0%                             | 10.0%                            | 10.0%                   |                         |         |         |
| Sucrose distearate                                                                 |                                                     |                                   | 20.0%                            | 20.0%                   | 10.0%                   | 20.0%   | 20.0%   |
| Glacial acetic acid                                                                |                                                     |                                   | 13.4%                            | 13.4%                   | 6.7%                    | 13.4%   | 13.4%   |
| Hydrated lime                                                                      |                                                     |                                   | 1.0%                             | 1.0%                    | 1.0%                    | 1.0%    | 1.0%    |
| Phenyl- $\alpha$ -naphthylamine                                                    |                                                     |                                   | 55.6%                            | 55.6%                   | 77.3%                   | 65.6%   | 65.6%   |
| Mineral lubricating oil (55 SUS at 210° F.)                                        | 82.0%                                               | 82.0%                             |                                  |                         |                         |         |         |
| Properties:                                                                        |                                                     |                                   |                                  |                         |                         |         |         |
| Appearance                                                                         | Uniform, homogeneous, opaque                        | Excellent, smooth, uniform grease | Excellent, smooth uniform grease | Soft semi-fluid         | No grease structure     |         |         |
| Stay-putness                                                                       | Does not flow down inclined surface or separate oil |                                   |                                  |                         |                         |         |         |
| Dropping Point, ° F.                                                               | Semi-fluid                                          | 500+                              | 500+                             | 500+                    |                         |         |         |
| Penetration ASTM 77° F., mm./10                                                    |                                                     |                                   |                                  |                         |                         |         |         |
| Unworked                                                                           | 400                                                 | 400                               | 225                              | 250                     | 275                     |         |         |
| Worked 60 strokes                                                                  |                                                     |                                   | 275                              | 275                     | 300                     |         |         |
| Worked 100,000 strokes                                                             |                                                     |                                   | 280                              | 290                     | 330                     |         |         |
| Water solubility                                                                   |                                                     | Insoluble                         | Insoluble                        | Insoluble               | Insoluble               |         |         |
| Norma Hoffmann Oxidation <sup>1</sup>                                              |                                                     | 320                               |                                  | 1,300 hrs. <sup>2</sup> | 414                     |         |         |
| Lubrication Life Hours <sup>3</sup> (250° F.-10,000 r.p.m.)                        |                                                     |                                   |                                  |                         | 1,000 hrs. <sup>4</sup> |         |         |
| Almen Test Wgts. Carried                                                           |                                                     | 15                                | 15                               |                         |                         |         |         |
| Four-Ball Wear Test (1,800 r.p.m.-10 Kg. Load 75° C.-1 hour) Scar Spot dia. in mm. |                                                     | 0.29                              |                                  | 0.26                    |                         |         |         |

<sup>1</sup> Hours to a 5 p.s.i. drop in oxygen pressure.

<sup>2</sup> Material still lubricating when test was discontinued.

<sup>3</sup> Anti-friction Bearing Manufacturers—National Lubricating Grease Institute test machine.

#### Example III

10.0 parts by weight of sucrose distearate was dispersed in 55.6 parts by weight of a mineral lubricating oil having a viscosity of 55 SUS at 210° F. by heating and stirring to 300° F. This base material was then allowed to cool. To the cool base (100-120° F.) was added 13.4 parts by weight of hydrated lime which was thoroughly dispersed in the ester dispersion to a smooth slurry. Then while stirring, 20.0 parts by weight of glacial acetic acid was added. Almost immediately a heavy solid grease structure formed. The temperature of reaction rose to 180° F. and stirring was continued until the temperature began to drop. External heating was then initiated and the temperature raised to 220° F. At this point a portion of the product was removed for testing. The balance of the grease was heated to 320° F. and then allowed to cool while stirring. At 200° F. on this cooling cycle, 1.0 part by weight of phenyl- $\alpha$ -naphthylamine was added to inhibit oxidation and the grease was allowed to further cool to room temperature.

#### Example IV

A grease was prepared in the same manner as the grease of Example III prepared at 320° F., except for different proportions of ingredients and the use of the monostearate in place of the distearate.

For comparison purposes a lubricant was prepared using calcium acetate as the sole thickener, i.e. without the ester. This lubricant was prepared as follows: 13.4 wt. percent of hydrated lime and 65.6 wt. percent of a mineral lubricating oil of 55 SUS viscosity at 210° F. was mixed to form an intimate slurry. Then 20.0 wt. percent of glacial acetic acid was slowly added while stirring, the temperature rising to 180° F. Heating was

45 As seen from the preceding table, Examples I and II show that both the sucrose mono- and distearate formed semi-fluid or soft greases. Example III (220° F.) demonstrated that calcium acetate monohydrate successfully further thickened the sucrose distearate-oil composition to a high melting point grease having good load-carrying ability, low wear and oxidation resistance. Example III (320° F.) shows that the anhydrous calcium acetate had substantially the same effect as well as demonstrating that such greases have a long lubricating life at elevated 50 temperatures. Example IV (320° F.) illustrates the use of anhydrous calcium acetate with sucrose monostearate. The comparison compositions A(220° F.) and A(320° F.) show the effect of calcium acetate monohydrate and anhydrous calcium acetate as the sole thickening agent.

55 Other esters of the invention may be used to prepare lubricants in the general manner of Example I. For example, Example I can be repeated but using cellobiose trioleate in place of the sucrose monostearate.

60 What is claimed is:

1. A lubricating grease composition comprising a major proportion of lubricating oil, about 5 to 30 wt. percent of an ester of one mole of a disaccharide and 1 to 3 moles of a C<sub>12</sub> to C<sub>32</sub> fatty acid and 5 to 40 wt. percent of an alkaline earth metal salt of a C<sub>2</sub> to C<sub>6</sub> fatty acid.

65 2. A lubricating composition according to claim 1, wherein said ester is a sucrose monoester of a C<sub>16</sub> to C<sub>24</sub> fatty acid.

70 3. A lubricating composition according to claim 1, wherein said ester is a sucrose diester of a C<sub>16</sub> to C<sub>24</sub> fatty acid.

75 4. A lubricating composition according to claim 1, wherein said ester is sucrose monostearate.

5. A lubricating composition according to claim 1, wherein said ester is sucrose distearate.

6. A lubricating composition according to claim 1,  
wherein said salt is calcium acetate.  
7. A lubricating composition according to claim 6,  
wherein said calcium acetate is anhydrous.

McLennan \_\_\_\_\_ Mar. 18, 1947  
Carmichael et al. \_\_\_\_\_ Aug. 14, 1951  
Sproule et al. \_\_\_\_\_ Aug. 19, 1952  
Clayton et al. \_\_\_\_\_ Jan. 18, 1955

## References Cited in the file of this patent

## UNITED STATES PATENTS

2,115,823 Miller et al. \_\_\_\_\_ May 3, 1938

2,417,428  
2,564,561  
2,607,735  
2,700,022

## FOREIGN PATENTS

Great Britain \_\_\_\_\_ Sept. 28, 1933  
Great Britain \_\_\_\_\_ Sept. 17, 1934